

## UNITED STATES PATENT OFFICE

ALBERT L. CLAPP, OF DANVERS, MASSACHUSETTS, ASSIGNOR TO BECKWITH MANUFACTURING COMPANY, OF BOSTON, MASSACHUSETTS, A CORPORATION OF MASSACHUSETTS

## BOX TOE

No Drawing. Original application filed October 31, 1922, Serial No. 598,214. Divided and application filed September 27, 1924, Serial No. 740,414. Again divided and this application filed March 10, 1927, Serial No. 174,424.

This invention has for its object to produce a shoe stiffener or sheet material from which such stiffeners may be produced.

Heretofore it has been customary in the manufacture of shoe stiffeners such as box toes to form a sheet of fibrous material, usually cotton and wool felt or like open porous material, and then to saturate or impregnate the sheet with a molten mass of a stiffening agent in the nature of hydrocarbons, which when cold is hard and friable but which when softened by a relatively moderate degree of heat permits the sheet or blank cut therefrom to become limp and flexible, so that the box-toe blank may be molded about the end of the last in pulling over or lasting the shoe. Various stiffening agents have been employed for this purpose, such as resins, gums, asphalts and hydrocarbons of the nature of Montan wax.

More particularly, the object of the present invention is to produce box toes or the sheets from which the box-toe blanks may be cut, by incorporating the stiffening agent with the pulp during the manufacture of the sheet in a paper machine so as to render unnecessary the step of separately impregnating the already formed sheet of fibrous material. It is necessary that the stiffening agent or agents should be thoroughly distributed throughout the sheet, that they should be of such nature that the box toe when molded is resilient and stiff, that they may be softened so as to render the sheet limp and flexible when heated to a relatively low temperature, and that they will set quickly when permitted to cool. One of the prime requisites of the sheet is that it must not part or tear easily when the stiffening agent is in a soft plastic condition, and that it may be stretched to some extent and pulled about the toe end of the last without being weakened or torn so as to conform to the shape of the last without injury.

The present invention consists of a box-toe blank, the sheet from which it is cut and a method of producing the same which will provide a box toe having the optimum characteristics which I have hereinbefore referred to.

In initially preparing the sheet, I employ a

furnish, including long fibers such as long rope fibers or flax fibers, and even in some cases may utilize long cotton fibers. In addition to these fibers, however, I also employ short fibers, preferably of the character of wood pulp used in the manufacture of paper,—this for the reason that a sheet formed only of long fiber is too open and porous and requires some shorter fiber in order to secure the necessary felting in the formation of the sheet on the paper machine. Inasmuch as an object which I desire to achieve is to secure a maximum quantity of stiffening agent in the sheet, it is necessary that the fibrous body of which the sheet is formed should be of such character that it will form properly in a web and yet be sufficiently open to permit the proper discharge of the water from the cylinder in the paper machine. An even web formation is secured by employing both the long fibers of the nature of cattle hair and short fibers such as obtained in the production of chemical wood pulp or such as obtained from waste kraft paper or the like. Of course, in lieu of wood pulp, one might employ rags or other raw material which provides relatively short fibers, which, when mixed with long fibers, will furnish a sheet having the desired characteristics.

As the thermoplastic stiffening agent I may utilize any gums or bituminous materials such as rosin, asphalt, Montan wax, copal or the like, which will give to the box toe the necessary stiffness and resiliency, and which will soften at a relatively low degree of heat and set quickly when cooled. Normally adhesive bituminous materials may likewise be utilized for furnishing the stiffening agents, provided they may be diluted with water and be thoroughly incorporated with the other elements or ingredients of the furnish in the beater stock.

As an example, one may proceed as follows: 8 parts by weight of long fibers such as rope, flax or cotton fibers and 8 parts by weight of sulphate pulp or equivalent short fibrous material may be placed in the beater with a large amount of water, much more than is ordinarily necessary for beating the stock. The beating engine is started in operation but

55

60

65

70

75

80

85

90

95

100

the knives are carefully adjusted so as not to cut the fibers but merely to brush them and secure a thorough, physically homogeneous mixture. The stock should be thinned with 5 water as this permits the rapid admixture of the ingredients. Of course, by taking a longer time, one might secure the same results with a thicker stock or one having less water. By having a very thin stock, it is possible to 10 secure the desired physical homogeneity in the course of 15 to 30 minutes. After the beater contents have been brushed as described, the thermoplastic stiffening agents may now be added. In the example herein 15 given, I employ 35 parts by weight of rosin, 25 parts by weight of gilsonite and 5 parts by weight of Montan wax, all pulverized to about 40 mesh. These ingredients are introduced into the beater, together with about 30 20 parts of asphalt emulsified or dispersed in water. This emulsion or dispersion preferably consists of normally adhesive asphalt emulsified or dispersed in water with a colloidal clay emulsifying agent, the asphalt 25 constituting the disperse phase of the emulsion. The amount of the emulsion added to the beaters is figured as the asphalt on a dry basis.

An emulsion, such as herein described, is 30 not per se my invention, and can be obtained on open market under the trade name of "K-B" emulsion.

With these hydrocarbon resinous ingredients, which constitute the thermoplastic stiffening agent, I preferably add a small amount 35 of casein dissolved in an alkaline solution. Instead of casein, I may use any other ingredient, which when precipitated by a precipitating agent carried down with it the stiffening 40 materials in a more or less conglomerate mass. Thus, in lieu of casein, I may use rosin size, viscous animal size, or other equivalent material. In some cases, however, I do not utilize either casein or the sizing material 45 last referred to, but ordinarily I find that it may be used with advantage. After these ingredients have been thoroughly intermixed with the fibrous material in the beater by continued rotation of the beater roll adjusted somewhat away from the bed plate, I 50 then add 10 parts by weight of alum as a precipitating agent. The fibrous stock with the stiffening agent thoroughly incorporated therein is now formed into a felted sheet by 55 a cylinder paper machine, and, when the sheet is of the desired thickness, it is cut and removed from the make-up roll. The sheet is then dried for the removal of water; and, when dry, is relatively open, free and porous 60 with free rosin, gilsonite, Montan wax and asphalt distributed as discrete particles throughout the sheet, and, when magnified, are visible as such. While still warm from the drier, the sheet is now preferably passed 65 through calender rolls heated to a sufficient

temperature to flux the hydrocarbon stiffening agents so that they will coalesce throughout the sheet. The effect of the calendering is further to condense and compact the sheet, so that, when the sheet cools, it is relatively 70 hard, compact or dense, stiff and resilient; and it is not affected by body temperature or materially affected by solar heat, but may be rendered limp and flexible at a temperature of 140° to 150° F.

It is quite evident that the particular ingredients, which I have mentioned in the foregoing example, may be changed or added to, although the furnish as described gives excellent results. For example, I may change 80 the fibrous ingredients by utilizing 5 parts by weight of long fibers such as flax, 5 parts by weight of sulphate pulp, and 5 parts by weight of the waste of the final sheet or waste which is produced from box-toe material as 85 ordinarily made.

In such case, the box-toe waste, which is the residue after cutting out the box toes or other shoe stiffeners, must be disintegrated before being added to the beater. I find that 90 this disintegration may be accomplished by subjecting the material to the action of an Abbe rotary cutter or grinder. Such machines are on the market and are easily procurable. Since there is some tendency of the 95 stiffening agents in the waste to gum the knives, I employ as a preventative a small amount of talc which may be thrown into the grinder from time to time by the handful. For example, I find that in any given amount 100 of the disintegrated waste fiber, there need not be over 1/2% of talc to insure the successful operation of the grinder. The disintegrated waste material consists of the usual fibers of which the felt was formed together with the 105 gums or solid hydrocarbons with which it was impregnated. It is possible to reduce the proportion of the asphalt emulsion from 30 parts by weight to, say, 20 parts by weight, and to increase the percentage of the casein 110 or other size which is employed.

By long continued experiment, I have found that a sheet, having only the asphalt emulsion as the stiffening agent, does not produce satisfactory box toes, for the reason that the sheet is too soft and does not possess the requisite rigidity and resiliency when cold, and that further it becomes too limp and soft when heated in the usual heaters employed in 115 shoe factories in connection with the pulling and lasting operations. I regard, however, the employment of the asphalt emulsion as desirable for the reason that the normally adhesive asphalt imparts a certain desirable toughness to the sheet when it is warm, and contributes towards permitting the box-toe 120 blanks to be folded and stretched about the last when the shoe is being pulled over or lasted. Since the asphaltic emulsion is insufficient to produce a sheet of necessary resil- 125

- iciency, rigidity and stiffness, I employ rosin, gilsonite or the equivalent which is distributed in the pulp in fine particles. In fact, instead of utilizing both rosin and gilsonite, I 5 may employ rosin alone, although I do not regard the final product as desirable as one in which these two ingredients are employed. Gilsonite, having a high melting point, adds stiffness and rigidity to the molded box 10 toe when subjected to body or solar heat. Inasmuch as the hydrocarbons must coalesce and become more or less amalgamated in the sheet, I use a certain proportion of Montan wax, which, because of its high degree of 15 penetrability when molten, acts as a fluxing agent for the other hydrocarbons in the sheet. The addition of Montan wax or like hydrocarbon of high penetrability and relatively low melting point is particularly desirable 20 when a tempering agent such as gilsonite is employed, as otherwise it may be necessary to heat the calendering rolls to such a high temperature to flux or coalesce the other hydrocarbon ingredients as might or would 25 tend to burn the long fibers employed in making the sheet. An advantage in employing - aseine rather than other size is that when precipitated with alum it is not affected by dry 30 heat but will soften when moist. Ordinarily, in the pulling over or lasting of shoes, in which stiffened box-toe blanks are employed, it is customary to subject the blank to moist heat, and therefore it is desirable to use some agent which when precipitated is not affected 35 by dry heat but which will soften when subjected to heat and moisture.
- After the sheet is finished, the blanks are cut and skived to serve as shoe stiffeners, such as box toes or counters.
- 40 The stiffening agents may be referred to as thermoplastic material, meaning to include by that term those compounds or mixtures which function as herein set forth,—namely those which may be incorporated in the wet 45 mass of fibrous material while in a finely divided condition, which soften on the application of heat not injurious to the shoe, which set rapidly when cooled, which give rigidity, stiffness and resiliency to the molded box 50 toe, and which will permit the heated and limp box-toe blank to be stretched about the toe end of the last, in the pulling-over and end-lasting operations.
- 55 This application is a division of my application Serial No. 740,414, filed September 27, 1924, which in turn is a division of my application Serial No. 598,214, filed October 31, 1922, and which issued on July 7, 60 1925, as Patent No. 1,544,813.
- What I claim is:—
1. A box-toe material, consisting of a fibrous pulp and a relatively longer vegetable fiber of the class described distributed 65 throughout the mass in felted relation there- with and impregnated with a thermoplastic binder.
2. A box-toe material, consisting of a fibrous pulp and relatively longer vegetable fibers of the class described distributed 70 throughout the same in felted relation therewith and impregnated with a thermoplastic binder, the proportion of vegetable fibers being no greater than that of the fibrous pulp.
3. A box-toe material, comprising a water-laid felt, consisting of rag pulp and much longer vegetable fiber distributed therethrough and in felted relation therewith, and impregnated with a thermoplastic binder.
4. In a water-laid felt, a fibrous foundation consisting of a rag pulp, and much longer vegetable fiber distributed throughout the mass in felted relation therewith, and capable of being impregnated with a thermoplastic binder.
5. In a water-laid felt, a fibrous foundation consisting of a rag pulp and relatively longer ligno-cellulosic fiber of the class described, uniformly distributed therethrough.
6. A felted fibrous foundation consisting 90 of about equal proportions of fiber of a length of the order of magnitude of rag or wood fiber and a fiber of a length of the order of magnitude of rope or flax fiber, said foundation being impregnated with sufficient 95 thermoplastic binder to be serviceable as a thermoplastic box-toe material.
- In testimony whereof I have affixed my signature.
- ALBERT L. CLAPP. 100
- 105
- 110
- 115
- 120
- 125
- 130